

(No Model.)

3 Sheets—Sheet 1.

J. REESE.

Process of Melting and Purifying Glass.

No. 240,846.

Patented May 3, 1881.



W<sup>W</sup>  
Witnessed  
J. M. Peters  
L. B. Krollin

Inventor Jacob Reese

(No Model.)

3 Sheets—Sheet 2.

J. REESE.

Process of Melting and Purifying Glass.

No. 240,846.

Patented May 3, 1881.



Witnessed  
J. M. Clegg  
H. B. Hallton —

Inventor Jacob Reese

(No Model.)

J. REESE.

3 Sheets—Sheet 3.

Process of Melting and Purifying Glass.

No. 240,846.

Patented May 3, 1881.



FIG. 4.



FIG. 5.

Wittendes  
H. M. Peters  
L. B. Moulton

Inventor Jacob Reese

# UNITED STATES PATENT OFFICE.

JACOB REESE, OF PITTSBURG, PENNSYLVANIA.

## PROCESS OF MELTING AND PURIFYING GLASS.

SPECIFICATION forming part of Letters Patent No. 240,846, dated May 3, 1881.

Application filed February 25, 1881. (No model.)

*To all whom it may concern:*

Be it known that I, JACOB REESE, a citizen of the United States, residing at Pittsburgh, in the county of Allegheny and State of Pennsylvania, have invented certain new and useful Improvements in the Process of Heating, Melting, Purifying, or Refining Glass or other Materials; and I do hereby declare the following to be a full, clear, and exact description thereof, reference being had to the accompanying drawings, in which—

Figure 1 indicates a front elevation of an improved plant adapted to the use of my improvement. Fig. 2 indicates a front elevation, partly in section, of the same. Fig. 3 indicates a plan view taken through at the line  $x-x$ , shown in Fig. 1. Fig. 4 indicates a cross-sectional elevation of the lower portion of one of the regenerators.

Like letters refer to like parts wherever they occur.

My invention relates to improvements in the process and apparatus for heating, melting, purifying, or refining glass or other materials; and it consists, first, in charging the material to be treated into a suitable furnace, vessel, or refining-chamber, and then subjecting it to the action of a column or currents of highly-heated air brought to a heating, melting, or refining temperature by being previously passed through a regenerator or other suitable air-heating apparatus, whereby the material may be heated, melted, purified, or refined in an open chamber by the aid of heated air alone, and without exposure to the deleterious effects of the impure gases and products of combustion; secondly, in an improved apparatus adapted to the use of my invention.

In the drawings, A and A' indicate the cylindrical regenerative stoves, which are placed above ground and connected to a heating, melting, or refining furnace, B, by means of intervening combustion chambers or stacks, C and C'. These combustion-chambers C and C' connect with the throats or necks of the opposite ends of the furnace B and extend up to the top of the domes of the regenerators A and A'. Each stove is covered externally with plate-iron, and is provided internally with a heating-surface composed of fire-brick in lattice-work arrangement, extending from a distributing-chamber at its base up to a point

near its dome, and occupying the entire cross-sectional area of the interior of the stove. These distributing-chambers extend through 55 the base of the stoves and project at both ends slightly beyond the walls of the regenerators. Openings provided with suitable valves, a a and a' a', are formed upon the side of the projecting ends of the distributing-chambers, for 60 the admission of air into the regenerators, and openings are provided on their opposite sides leading to the stack-flue, and having suitable valves, a<sup>2</sup> a<sup>2</sup> and a<sup>3</sup> a<sup>3</sup>, to regulate the passage of the waste gases out from the distributing-chambers. The distributing-chambers are 65 also provided with doors at both ends to admit of cleaning, &c.

D indicates the melting-chamber or part of the furnace which is lined with pot-clay, such 70 as is in common use for the manufacture of pots for glass-making.

Beneath the refining-chamber or hearth is located a gas-flue, E, the opposite ends of which terminate in a series of fire-brick flues, 75 leading up into the base of the combustion-chambers C and C', as indicated in Figs. 2 and 3. The gas-flue E is connected at its center with a gas-main, E', leading to the gas-producers, and is provided with valves e and e', 80 for the admission of gas alternately into either of the combustion-chambers.

In constructing the plant which I have just described, I prefer to form a slight depression or hollow in the lining of the pot of the refining-chamber immediately in front of each of the charging or gathering doors, as the effect of providing such depressions will be that when the material is melted and refined it will run into the depressions from the other portions of the refining-chamber or pot, and may be more readily gathered and removed from the furnace. The furnace may also, if desired, be provided with suitable tuyeres projecting into the pot, for the admission of hot blast into and through the material to be treated, for the purpose of accelerating the melting of the charge. In this case, however, the action of the blast should be stopped after the material is melted, in order that it may remain at a state of rest 90 for the emission of any occluded gases and for its more thorough refining.

In operating the plant the air-valves a a of the regenerator A are opened and its stack-

valves  $a^2$   $a^2$  are shut, the stack-valves  $a^3$   $a^3$  of the opposite stove, A', are opened, and its air-valves  $a'$   $a'$  are closed. Both gas-valves  $e$  and  $e'$  of the gas-flue E are shut, and air is then forced into the regenerator A through the air-valves  $a$   $a$ , under a slight pressure, until the current has passed over the refining-chamber of the furnace. The gas-valve  $e'$  is then opened and gas is forced into the combustion-chamber C', where it unites with the air which has passed over the refining-chamber. Combustion takes place and the flame and products of combustion pass upward in the combustion-chamber into and through the regenerator A', and out through the valves  $a^3$   $a^3$  into the stack. After about twenty minutes (more or less) the regenerator A' has become highly heated, and the gas-valve  $e'$  is closed, and, as the air continues to flow, in a moment or two the gases and products of combustion are driven, by the current of air, out of the regenerator A' into the stack. The air-valves  $a$   $a$  are then closed and the stack-valves  $a^2$   $a^2$  of the regenerator A are opened and the air-valves  $a'$   $a'$  are opened, and the stack-valves  $a^3$   $a^3$  of the regenerator A' are shut, the gas-valve  $e'$  is closed and the valve  $e$  of the gas-flue E is then opened, thus reversing the currents, and the air entering the regenerator A' becomes highly heated, passes down the combustion-chamber C' and over the refining or melting chamber, and enters the combustion stack or chamber C, where it unites with the gas and an internal and vivid combustion takes place, and the flame and products of combustion pass upward into and through the regenerator A, and then outward through the stack-valves  $a^2$   $a^2$  into the stack. The currents are thus reversed every twenty or thirty minutes, until the furnace becomes thoroughly heated to about 2,000° Fahrenheit. When the furnace has acquired a temperature of 2,000°, the glass material may be charged through the doors and the doors closed. In from two to three hours the glass will be thoroughly melted and an additional charge of glass material may then be charged, so as to more fully fill the pot, which will be melted in from one to two hours. The heat should now be increased to about 3,000° Fahrenheit, and continued after the ebullition ceases for about three or four hours, so as to keep the glass in a highly-fluid condition and a state of rest, in order that the gases may escape and the resulting glass be free from blow-holes or bubbles. When the glass is thus thoroughly melted and refined, the temperature is lowered by shutting off a portion of the air and gas, for the purpose of reducing the glass to the viscid state required for gathering. The gathering-holes may then be opened and the glass withdrawn in the usual manner. The time required for melting and refining a heat in such a regenerating-furnace will be twelve (12) hours, so that the glass material may be charged at six o'clock in the evening and be ready to draw at six o'clock the following morning.

Care should be taken in reversing the cur-

rents that the gas-valves should be first closed, and the air passing over the hearth be permitted to drive all of the gas out of the regenerators before the air-valves are changed. The current of air should also be reversed over the refining-chamber before the gas-valve be opened. Hot air only passes over the refining-chamber, and the hot air is thus utilized before it is used for combustion, and the gas or the gases resulting from combustion never enter the refining-chamber, but are utilized for heating the regenerators only.

The advantage of this process is that glass may be melted and refined and other material treated, melted, or refined in an atmosphere of hot air without the products of combustion coming in contact with the glass or other material under treatment; and glass which now requires thirty-six hours to melt it and refine it in closed pots may be melted and refined by the use of my process of hot air in twelve hours, and be made freer from bubbles or other defects than the glass melted in closed pots, because I can produce a higher heat and make the glass more fluid, and thus more thoroughly refine it in one-third of the time. In open pots, as at present practiced, where the glass is subject to sulphur and other gases of combustion, it takes twelve hours to melt the most fusible common mixture of bottle-glass and twenty-four hours to melt common window-glass. Thus I am able to secure all the advantages of the closed pot, which requires thirty-six hours to a heat in the shortened time now required for melting common bottle-glass.

When the product is to be used for plate-glass, an adjustable pot could be used and the melting be done by blowing the hot air through the material, as cold air is now blown through the metal in the Bessemer converter, and when the glass has been melted the pot can be turned over on its side and the hot air blown over the glass until it is sufficiently refined and ready for use. The pot could then be turned down and the glass run out on the plate and rolled, and afterward treated as now in common use or practice; or the furnace containing the pot could be made adjustable, and after the glass had been prepared, as first described, the pot or furnace containing the pot could be turned so as to cause the glass to run out on the plate; or adjustable open-mouth pots may be placed in a furnace and heated with air until the material is melted and the glass is refined. The pots may then be withdrawn through the door and emptied on the plate.

I have described the operation of my improvement as applied to the manufacture of glass; but I do not intend to limit its use solely to such purpose, as it is applicable to many other purposes wherein it is desirable that the material to be heated, melted, purified, or refined should not be subjected to the deleterious effects arising from combustion or the presence of sulphurous gases and products of combus-

tion present in the furnace or refining-chamber, and as a high heat may be developed by the use of hot air alone in the refining-chamber, my improvement will be applicable generally to refining purposes.

Having described my invention, what I claim, and desire to secure by Letters Patent, is—

1. The process herein described of heating, melting, and refining glass and other material, which consists in charging the material to be treated into a suitable refining vessel or chamber, and then subjecting it to a high and continuous temperature by means of a column or currents of highly-heated air forced into, through, or over the material contained in the refining-chamber, whereby the material may be heated, melted, purified, or refined without exposure to the deleterious effects of sulphurous gases and mechanical impurities contained in the products of combustion, substantially as hereinbefore specified.

2. The method herein described of heating, melting, purifying, or refining materials for the manufacture of glass or other purposes, which consists in charging the material into a suitable refining vessel or chamber, and then subjecting it to a high and continuous temperature obtained solely by means of a current of air raised to the required temperature by its passage through a highly-heated regenerator, and without the presence of combustion or the products in the refining chamber or vessel, substantially as specified.

3. In the process of heating, melting, refining, or purifying materials for the manufacture of glass or other materials, the method herein described of freeing the regenerator from the presence of waste gases and products of combustion, which consists in closing the gas-valve for a short time previous to the reversal of the air-current, whereby the waste gases are driven

from the regenerator into the stack and their presence in the refining-chamber on the reversal of the air-current is avoided, substantially as herein specified.

4. The improved plant herein described, which consists of two cylindrical regenerative stoves placed above ground and provided with exterior combustion-chambers, which communicate with the top of their domes and with the opposite ends or necks of a heating, melting, or refining chamber, substantially as herein specified.

5. The combination of two regenerators, each provided with a vertical combustion-chamber, an intervening melting or refining chamber, and a gas flue or conduit connecting with each combustion-chamber, and provided with valve or valves arranged substantially as specified, so that the gas may be directed into either combustion-chamber, to combine with the air which has passed over the melting or refining chamber, substantially as and for the purpose specified.

6. The method herein described of utilizing the waste heat in melting and refining processes, which consists in, first, causing the highly-heated air-currents from a regenerator to pass through a melting or refining chamber, whereby a portion of the heat is utilized, and, secondly, combining gas therewith and inducing combustion after the air has passed the melting-chamber, either in or before the same has reached the regenerator, whereby the residual heat of the air is utilized, substantially as and for the purpose specified.

In testimony whereof I have hereunto set my hand this 24th day of February, 1881.

JACOB REESE.

Witnesses:

F. W. RITTER, Jr.,  
H. B. MOULTON.